

## UNITED STATES PATENT OFFICE

1,931,251

TORSION-SPRING FOR CLOCKS, WATCHES,  
ETC.

Thomas H. Chamberlain, New Haven, Conn., assignor to The New Haven Clock Company, New Haven, Conn., a corporation

No Drawing. Application March 17, 1930  
Serial No. 436,650

## 2 Claims. (CL. 75—1)

This invention relates to an improvement in torsion-springs for various measuring or indicating instruments-of-precision, such as clocks, watches, ammeters, voltmeters, and other instruments in which a variation in the modulus of elasticity of the torsion-springs, due to thermal changes, is a factor affecting accuracy.

The main object of my invention is to produce a torsion-spring which will have a substantially-uniform modulus of elasticity throughout the normal range of atmospheric temperatures, whereby thermal changes will not appreciably affect the precision of the readings of an instrument in which my improved torsion-spring is installed.

A further object of my invention is to produce a torsion-spring having a substantially-uniform modulus of elasticity throughout the normal range of atmospheric temperatures, and which is sufficiently ductile to be readily drawn, rolled, or otherwise formed and shaped.

A further object of my invention is to produce a torsion-spring characterized as above which will be highly resistant to corrosion.

With the above and other objects in view, as will appear from the following, my invention consists in a torsion-spring having a substantially-uniform modulus of elasticity throughout the normal range of atmospheric temperatures and consisting of an alloy hereinafter described.

My improved torsion-spring is preferably made from a ferrous alloy of the following composition:

|           | Per cent       |
|-----------|----------------|
| Carbon    | 0.15 to 0.17   |
| Manganese | 0.70 to 0.90   |
| Silicon   | 0.65 to 0.80   |
| Nickel    | 35.50 to 36.50 |
| Chromium  | 12.00 to 13.00 |

Iron to form the balance after a suitable allowance for impurities, such as sulphur, phosphorous, etc.

The carbon- and manganese- and silicon-content set forth above act as hardeners, and while they, in the aggregate, are appreciably high, it will be noted that no single one of them is sufficiently high to occasion brittleness, which might result, were a single hardener to be employed. For instance, by employing both manganese and silicon, in addition to carbon, to secure the desired hardness, the carbon may be kept at such a small percentage as not to occasion any appreciable formation of chrome-carbides.

A torsion-spring composed of my improved

alloy is not only comparatively easy to form, but its tension is so nearly uniform, despite normal thermal changes, that when employed as a balance- or hair-spring in a watch or clock it insures substantially-uniform impulses to the balance-wheel of the time-piece with which it is employed, so that all other variable factors having been provided for, approximately perfect time-keeping results.

While I have set forth the above alloy as being the preferable one, I am satisfied from repeated experiments that the nickel- and chromium-content is the controlling factor in imparting the substantially-uniform modulus of elasticity to my improved torsion-spring, and I wish to have it understood that I do not limit myself to an alloy other than that defined in the claims.

I claim:

1. A torsion-spring combining high elastic limit, ductility and a substantially-uniform modulus of elasticity comprising the following elements within the ranges given:

|           | Per cent       |
|-----------|----------------|
| Nickel    | 34.50 to 37.50 |
| Chromium  | 11.00 to 13.00 |
| Manganese | 0.60 to 1.00   |
| Silicon   | 0.25 to 0.90   |
| Carbon    | 0.07 to 0.35   |

Iron forming substantially all of the balance

2. A torsion-spring combining high elastic limit, ductility and a substantially-uniform modulus of elasticity comprising the following elements within the ranges given:

|           | Per cent       |
|-----------|----------------|
| Nickel    | 35.50 to 36.50 |
| Chromium  | 11.50 to 12.50 |
| Manganese | 0.70 to 0.90   |
| Silicon   | 0.65 to 0.80   |
| Carbon    | 0.07 to 0.17   |

Iron forming substantially all of the balance

THOMAS H. CHAMBERLAIN.

100

105

110